

Nov. 21, 1939.

E. W. DUNBAR

2,180,924

RUBBER FOOTWEAR

Filed Feb. 24, 1937

4 Sheets-Sheet 1



Fig. 2



Fig. 1



Fig. 3



Fig. 5



Fig. 4

INVENTOR  
Ernest W. Dunbar  
BY J. H. McCready  
his ATTORNEY

Nov. 21, 1939.

E. W. DUNBAR

2,180,924

RUBBER FOOTWEAR

Filed Feb. 24, 1937

4 Sheets-Sheet 2



INVENTOR  
Ernest W. Dunbar  
BY J. McCreedy  
his ATTORNEY

Nov. 21, 1939.

E. W. DUNBAR

2,180,924

RUBBER FOOTWEAR

Filed Feb. 24, 1937

4 Sheets-Sheet 3



INVENTOR  
Eugene W. Dunbar  
BY J. H. Mc Cready  
his ATTORNEY

Nov. 21, 1939.

E. W. DUNBAR

2,180,924

RUBBER FOOTWEAR

Filed Feb. 24, 1937

4 Sheets-Sheet 4



*Fig. 16*



*Fig. 17*



*Fig. 15*



*Fig. 18*

INVENTOR  
Ernest W. Dunbar  
BY J. & W. Cready  
his ATTORNEY

## UNITED STATES PATENT OFFICE

2,180,924

## RUBBER FOOTWEAR

Ernest W. Dunbar, Hudson, Mass., assignor to  
 Cambridge Rubber Co., Cambridge, Mass., a  
 corporation of Massachusetts

Application February 24, 1937, Serial No. 127,426

4 Claims. (Cl. 36—14)

This invention relates to rubber soled shoes and to the parts of such shoes. It is more especially concerned with the bottom structure of footwear of this type.

5 Objections often raised to the use of rubber shoes are the facts that they "burn" the bottoms of the feet of some individuals, or cause the feet to sweat excessively, and the further fact that these shoes are relatively heavy. On 10 the other hand, a large proportion of the purchasing public prefers shoes with rubber bottoms because of the cushion effect which they afford, the better grip on the ground which they give, and their superior waterproof and wearing 15 properties.

The present invention aims to improve rubber-soled shoes with a view to eliminating the objectionable features above mentioned, while still preserving the advantages of footwear of 20 this type.

The nature of the invention will be readily understood from the following description when read in connection with the accompanying drawings, and the novel features will be particularly 25 pointed out in the appended claims.

In the drawings,

Figure 1 is a perspective view of an outing or beach shoe embodying features of this invention;

30 Fig. 2 is a vertical, sectional view of a portion of the sole structure of the shoe shown in Fig. 1;

Fig. 3 is a similar view through the entire bottom of the shoe;

35 Fig. 4 is a transverse, sectional view through the forepart of the shoe;

Fig. 5 is a side view of a portion of the binder strip used on the outsole;

40 Figs. 6 and 7 are perspective and edge views, respectively, illustrating steps in the process of manufacture of elements of the shoe bottom;

Fig. 8 is an edge view showing a further step in this process;

45 Fig. 9 is a perspective view of a man's shoe including a bottom embodying features of this invention;

Fig. 10 is a vertical, sectional view showing a different type of shoe bottom embodying the invention;

50 Figs. 11 and 12 are perspective views of the bottom and top, respectively, of a combined sole and heel constructed in accordance with the invention;

55 Figs. 13 and 14 are sectional views on the lines 13—13 and 14—14, respectively, Fig. 10;

Fig. 15 is a perspective view of another shoe embodying this invention;

Figs. 16 and 17 are vertical, sectional views through the forepart and heel part, respectively, of the shoe shown in Fig. 15; and

Fig. 18 is a fragmentary, vertical, sectional view showing features of another form of the invention.

Referring first to Figs. 1 to 4, inclusive, the shoe there shown comprises an upper 2, an 10 insole 3, and an outsole, which is indicated in general at 4. The upper may be of any suitable character such as fabric, leather, or combinations of these materials. As above indicated, the greater part of the weight of a shoe 15 is in its bottom structure. In most shoes it is necessary to have a bottom of considerable thickness in order to prevent the foot from feeling too plainly the irregularities in the ground, to provide better heat insulation, and to avoid excessive 20 flexibility in the shoe bottom. According to the present invention, these desirable characteristics are obtained, while still producing the necessary wearing qualities and avoiding excessive weight, by using in the bottom structure a high percentage of sisal fiber. In the 25 particular shoe shown the insole 3 consists essentially of a layer of sisal fibers loosely matted together but held in cooperative relationship to each other through the use of a limited quantity of a waterproof binder. This may, for example, be rubber, or it may consist of some cellulose ester, such as cellulose acetate, dissolved in a suitable solvent. Or, binders may be dispensed with, and the body of fiber may be mechanically bound together as, for example, by superposing a flexible top sheet *a*, Fig. 1, on the layer of fibers, and stitching this and said layer together, preferably with a fabric bottom sheet.

The outsole, as shown in Fig. 3, is composed 40 of an upper section *c* and a lower or tread layer *d*. The upper section consists of a body of sisal fiber either made of ply structure or not, as desired, and containing a sufficient proportion of rubber, or other waterproof binder, to bond the 45 fibers securely together but without materially

decreasing the porosity or reducing the volume of the voids in this member. The top and bottom surfaces of this sisal fiber layer, however, are sufficiently coated with a high grade gum 50 rubber compound so that they will readily unite with the adjacent members of the bottom. In order to produce an edge having a more attractive appearance than that presented by the ends of the fibers, the entire edge surface is 55

covered with a binder strip 5 which is initially coated with a rubber and therefore bonds securely to the rubber content of the sisal fiber assembly. The nature of this binder strip necessarily will be determined by the character of the shoe in which it is to be used. For some purposes it will simply be a strip of rubber compound. In other shoes, such for example as that shown in Fig. 1, it is preferable to use a fabric binder of some such nature as that illustrated in Fig. 5, the color and texture of which will contribute to the general design of the shoe. The tread layer *d* may be made of any suitable rubber composition which will give the desired wearing qualities. It also may be colored, embossed, or ornamented in any suitable manner.

In making this shoe the usual procedure is to make and stitch together the parts of the upper in the usual manner, and then to perform the shoe making operations on a last, the various parts of the bottom having previously been manufactured. Usually the insole 3 is first secured to the bottom of the last, its margins are coated with cement, and the upper is lasted over upon these margins in the same manner as in making rubber footwear of the orthodox types. Next a rubber welt 6 is cemented entirely around the lower margin of the insole 3, and a friction binder sheet 7 is cemented to the bottom of the insole, provided this strip has not been included in the insole structure. In the latter event, it is coated with cement at this stage of the process. The sisal fiber assembly *c* now is properly registered with the edges of the shoe and is laid upon the bottom of the insole and the overlasted margins of the upper, after which the tread layer *d* is similarly registered with and applied to the bottom of the section *c*. If the parts have been assembled while the rubber elements are in an unvulcanized condition, then the shoe will be subjected to vulcanization. On the other hand, if the parts when assembled are in a vulcanized or self-vulcanizing state, then the vulcanizing step may be eliminated.

Usually the former practice is preferred.

While the sisal section of the outsole may be made in various ways, the preferred method consists in working the long sisal fibers into the form of a layer or sheeted body having considerable thickness, say for example, three-eighths of an inch or a half inch. Such a body is illustrated at 10 in Fig. 6. This operation can be performed by hand or in various kinds of fiber working machinery designed for the purpose of manipulating fibers and presenting them in a sheeted or bat form. In such a sheeted body the fibers are not arranged in any definite relationship to each other, but are disposed promiscuously, the fibers being so distributed, however, that when the mass is compressed a sheet or layer of substantially uniform thickness will be produced. In this connection it may be pointed out that while sisal is the preferred fiber, hemp can also be used satisfactorily. The textile fibers and others of a similar nature, however, are distinctly inferior.

The sheeted stock produced in the manner above described is next impregnated with a binder adapted to bond the fibers together permanently. A flexible waterproof binder should be used for this purpose and the best material which I have been able to find is a rubber binder such as rubber latex, either vulcanized or unvulcanized. In some cases, however, other binders, such as those of an asphaltic nature, or those made from synthetic gums, resins, or balsams, may be em-

ployed. The impregnating step may be performed in any convenient manner as, for example, by running the sisal fiber bat through the liquid binder and then through squeeze rolls to remove the surplus, after which the bat should be dried to evaporate the solvent or other dispersing agent used. If latex is used for this purpose in the ordinary concentrations, the bat will pick up approximately its own weight of rubber. In other words, after the water or serum has been evaporated, the impregnated sheet will have gained approximately its own weight of dry rubber. The proportion of binder so added to the bat can, however, be controlled by suitably varying the concentration of the impregnated bath.

The impregnating, squeezing, and drying operations above described compresses the bat so that its final thickness may be perhaps one-quarter or one-half of that of the original bat. The material at this stage of the process is indicated at 11 in Fig. 7. Usually it is desirable to apply a calendar coat of rubber to one side of the sheet 11, as shown at 12 in Fig. 8, and for most purposes a spreader coat 13 of rubber is subsequently applied to the uncoated side of the sheet. In making insoles a sheet of the material which is to form the upper surface of the insole may then be combined with the layer shown in Fig. 8. Also, in these calendaring and spreader coating operations the layer is further consolidated to bring it down to the desired dimensions, the final thickness being so predetermined that the layer will have the necessary degree of mechanical strength, porosity and resistance to compression.

The sheeted layer of sisal fiber produced in the manner above described is a highly porous, open, reticulated structure through which air flows very freely, the proportion of binder added to the original fiber being so limited that the fibers are united chiefly at their intersections with each other, but the interstitial spaces are not substantially reduced. In this connection it may be pointed out that in making the insole 3 the layer 11, as shown in Fig. 7, is sometimes used.

In making soles or heels several processes may be followed. For example, the uncoated but impregnated layers 11 may be completely filled with rubber and either vulcanized, or partially vulcanized, depending upon the subsequent shoe making processes. At any convenient stage in this procedure the plies may be secured together to produce soles and heels of the desired thickness as illustrated at 8 and 9 on the shoe shown in Fig. 9. Here the soles and heels are solid, but a high proportion of the rubber has been displaced by sisal fiber and the presence of these fibers at the bottom or wearing surfaces of these members greatly reduces the tendency of the rubber to slip on a wet surface.

According to the method usually preferred, the sisal layers 11 are coated on one or both sides and then the desired number of them are superposed, one on another, necessary to build up a structure of the required thickness for the heel or sole (both these elements being hereinafter included, where the context permits, in the term "outsole"). Sole and heel blanks may be cut out of such an assembly with the usual cutting dies, and the heel blanks may be applied to the heel ends of the sole blanks, as shown in Fig. 10, the sole blank being indicated at 14 and the heel blank at 15. These parts will be secured to each other by the rubber coating or coatings which they carry. Subsequently a tread layer 16 of a suitable rubber composition is applied to the outer

surface of this entire assembly and secured there to by the inherent adhesiveness of these parts or by suitable rubber cement. Also, an edge covering or binding strip 17 of rubber preferably is applied to this whole assembly, this strip being cut to size and shaped preparatory to being applied, one edge *f*, Fig. 11, being registered with the inclined breast of the heel portion of the outsole and then the strip being extended around the heel and the forepart and the final edge *g* abutted against the edge *f*. This binder overlaps both the sisal and the rubber plies and is folded over upon the upper surface of the sisal section 14, as clearly shown in Fig. 12.

The outsole assembly produced in the manner just described is then ready to be applied to the bottom of such a shoe as that shown, for example, in both Figs. 9 and 15. The latter shoe is of the outing type, usually made with a fabric upper, and the upper and outsole are secured together partly by the union of the rubber constituents of the insole and outsole and partly through the medium of a welt strip 18 like that shown at 6 in Figs. 1 to 4. During the vulcanizing operation this welt bonds securely to or unites with the folded-over portion of the cover strip 17 on the upper surface of the outsole assembly and these two parts thus cooperate to form a continuous rubber member uniting the tread ply 16 of rubber with the upper of the shoe. Thus all the exposed surfaces of the sisal body are completely covered with rubber.

Sections of the shoe shown in Fig. 15 are illustrated in Figs. 16 and 17, the upper being indicated at 20 and the insole at 21. A sisal filler strip 22 may or may not be used, as desired.

In some cases it is preferable to run the tread strip 16 for the sole directly through the heel and then to mount the heel on top of this strip. Such an arrangement is illustrated in Fig. 18 where the sisal layer is shown at 14' and the tread layer of the sole at 16', this latter layer extending the entire length of the sole. The heel includes a sisal section 15', a tread section 23 of rubber, and an edge covering strip 24 also of rubber. In this arrangement, therefore, the sisal body 15' is completely enclosed at top, bottom and sides by rubber. Preferably a stiffer sheet of material 19, Figs. 10 and 14, loaded with rubber is placed at the bottom of the heel above the tread layers 15 or 16 where it serves to reinforce the tread layer.

It should be observed that in all these shoes a high proportion of the volume of the bottom structure consists of sisal fiber. Consequently, such a shoe may be made extremely light in weight while still having exceptionally good heat-insulating properties, ample resiliency to give the cushioning properties which are one of the important advantages of rubber shoes, and while preserving, also, the surer grip on the ground or sidewalk which a rubber tread affords. Inasmuch as the sisal fiber in such shoes as those shown in Figs. 1 and 15 holds a relatively thick

body of air immediately under the foot, and a limited amount of interchange of this air naturally occurs in walking due to the resiliency of the sisal structure, better ventilation for the foot is produced than in ordinary shoes, and the tendency to "burn" the bottoms of the feet or to make them sweat excessively, is obviated. In fact, the shoe is extremely cool in hot weather. The shoe bottom also has the same wearing and waterproof characteristics as prior rubber soled shoes of corresponding types. Moreover the sisal layers are of advantage in imparting to the sole added strength and the degree of stiffness necessary to counteract the excessive flexibility of the rubber. In addition, the expense of manufacture of a shoe of this character is less than that of shoes of corresponding grades made by the usual rubber shoe methods.

Having thus described my invention, what I desire to claim as new is:

1. A shoe comprising an upper, an insole, and a rubber tread member united thereto, a high percentage of the volume of said tread member consisting of a layer of sisal fibers loosely matted together but secured to each other by a flexible binder, the proportions of said binder being so limited that said layer maintains a relatively thick body of air under the foot, and a rubber connection between the tread member and the shoe upper.

2. A shoe comprising an upper, an insole, and an outsole united thereto, said outsole comprising a relatively thick layer of sisal fibers loosely matted together but secured to each other by a flexible waterproof binder, the proportions of said binder being so limited that said layer maintains a relatively thick body of air under the foot, a rubber tread layer permanently secured to said sisal layer, and a rubber connection between the tread layer and the shoe upper.

3. A shoe comprising an upper, an insole, and an outsole united thereto, said outsole comprising a relatively thick layer of sisal fibers loosely matted together but secured to each other by a flexible binder, the proportions of said binder being so limited that said layer maintains a relatively thick body of air under the foot, a rubber tread layer permanently secured to said sisal layer, and a rubber strip covering the edge of said sisal layer and united with said rubber layer and connected to the shoe upper.

4. A shoe comprising an upper, an insole, and an outsole united thereto, said outsole comprising a relatively thick layer of sisal fibers loosely matted together but secured to each other by a flexible waterproof binder, the proportions of said binder being so limited that said layer maintains a relatively thick body of air under the foot, a rubber tread layer permanently secured to said sisal layer, a rubber strip covering the edge of said sisal layer and united with said rubber layer, and a rubber welt strip connecting said edge covering strip with the upper of the shoe.

ERNEST W. DUNBAR.